

## UNITED STATES PATENT OFFICE

2,196,750

## YARN CONDITIONING PROCESS

Joseph B. Dickey and James G. McNally, Rochester, N. Y., assignors to Eastman Kodak Company, Rochester, N. Y., a corporation of New Jersey

No Drawing. Application December 16, 1938,  
Serial No. 246,207

14 Claims. (Cl. 28—1)

This invention relates to the treatment of cellulose organic derivative filaments, fibers, threads and the like and more particularly to a method of eliminating the tendency of such materials to accumulate charges of static electricity in twisting, winding and spinning. The invention also relates particularly to the treatment of cellulose organic derivative cut staple fibers to adapt them for the manufacture of spun yarns.

- 10 As is well-known, cellulose organic derivative materials, particularly in filament, yarn, or sheet form, are particularly subject to the accumulation on their surfaces of charges of static electricity from frictional and other influences. In 15 the case of filaments and yarns in which the surface area of the material (per unit of weight) is enormously greater as compared to sheets or films, the problem of static often assumes serious proportions. In the manufacture of yarns of various 20 types from artificial filaments, numerous steps in which the yarn is subjected to frictional influences may be necessary, as for example, twisting, winding, warping, carding, combing, drawing, spinning and the like, all of which operations 25 tend to produce large accumulations of static on the filaments. This is particularly aggravated in the utilization of cut staple, as for example, in the making of spun yarn, since in carding and combing considerable friction is developed and as 30 a result sufficient charges accumulate on the fibers to make the formation of the web difficult, if not impossible; furthermore, even if a web is formed with some degree of success, the subsequent drafting operation produces a very uneven 35 spun yarn or intermediate roving due to the presence of the static charge. In addition, there is the ever-present fire hazard.

Cellulose derivative yarn, particularly in the form of cut staple, is extremely difficult to handle in the various operations involved in making spun yarn, not only because such material is composed of filaments having smooth, glass-like surfaces without natural kink or irregularity, but also because it has relatively negligible moisture 45 content at normal humidities, as compared to natural fibers such as cotton and wool, making it inherently far more susceptible to the accumulation of static. The charges accumulating on cellulose derivative cut staple fibers are, under some 50 circumstances, even sufficient to separate the individual fibers a distance of inches; notwithstanding their relatively minute size.

This invention has as its principal object to provide an improved method for the treatment 55 of cellulose organic derivative yarns to reduce or eliminate the tendency of such yarns to accumulate charges of electricity under frictional and other influences. A further object is to provide a method of facilitating the handling and employment of cellulose organic derivative cut staple

fibers in the various operations involved in the manufacture of spun yarns. A still further object is to provide a method of treating cellulose organic derivative yarns in either filament or cut staple form, wherein the material is simultaneously softened and lubricated and the accumulation of static charges thereon is prevented. Another object is to provide an improved type of cellulose organic derivative cut staple having little or no tendency toward accumulation of static electrical charges. Other objects will appear hereinafter.

These objects are accomplished by the following invention which in its broader aspects comprises applying to cellulose organic derivative yarns either in the form of filaments, threads or staple fibers, an antistatic composition characterized by the presence therein of organic amine salts of furfuryloxy and tetrahydrofurfuryloxy aliphatic acids, having the general formulas:



and



where A is a substituent selected from the group consisting of hydrogen, substituted and unsubstituted alkyl groups, n is 1, 2, etc., and x is 1, 2, etc. The structure of these salts may be represented by the formulas:



and



where A, x, n have the meaning previously referred to, and B is a primary, secondary, tertiary or quaternary organic base, or ammonia.

The various amine salts of the above mentioned acids may be prepared by any of the known methods for preparing relating compounds. As a rule we prefer to treat the desired amine with a stoichiometric amount of the acid or in certain cases an excess of the acid or amine may be used.

In accordance with our invention the above mentioned amine salts may be applied to the 55 yarn in any convenient manner, for example, by roll, wick, immersion, spraying or the like. Inasmuch as these compounds are soluble in oil they may be dissolved or dispersed in oils such as mineral oil, blown and unblown, drying, and semi-

5

10

15

20

25

30

35

40

45

50

55

60

drying, vegetable and animal oils, examples of which are light mineral, neat's-foot, olive, teaseed, castor, soya bean, rapeseed oils, etc.

In the following examples and description, we have set forth several of the preferred embodiments of our invention, but they are included merely for purposes of illustration and not as a limitation thereof.

*Example 1*

10. Tetrahydrofurfuryloxy acetic acid sodium salt is applied to textile materials (silk, cotton, wool, viscose, cellulose acetate, etc.) by means of a bath, wick, roller, spray, etc. to facilitate their knitting, weaving, spinning and the like. Yarns 15 treated with the above type of agent are of special value in the preparation of cut staple fibers. These fibers may be oiled before or after cutting.

*Example 2*

20. A conditioning liquid is made up as follows:

- Parts  
Ditetrahydrofurfurylamine propionate 70  
25 Furfuryloxyacetic acid oleyl amine salt 30  
and applied to textile materials such as silk, wool, cellulose acetate, etc. as described in Example 1. If the yarn is intended primarily for knitting, the amount of conditioning liquid applied may vary from 4-25% by weight of the yarn, and if for weaving between 1-5% by weight of the yarn.

35 Cellulose acetate filaments treated as described above are quite soft and pliable and give improved results in various textile operations such as weaving, knitting, etc., and especially in the production of cut staple fibers.

Conditioning liquids particularly useful for the treatment of various types of yarns in accordance with our invention particularly those composed of or containing cellulose acetate, cellulose acetate propionate, cellulose acetate butyrate, and similar organic acid esters, and especially adapted for the de-electrification or anti-static treatment of cellulose organic derivative cut staple yarns are as follows:

*Example 3*

- Parts  
50 5-methyltetrahydrofurfuryloxyacetic acid methylamine salt 1  
Olive oil 40  
Glycerol acetone butyrate 59

*Example 4*

- 55 5- $\omega$ -hydroxymethylfurfuryloxyacetic acid diethylamine salt 5  
Blown olive oil 60  
Glycerol methyl ethyl ketone 35

60 *Example 5*

- Parts  
85  $\beta$ -tetrahydrofurfuryloxy propionic acid-tri-propylamine salt 5  
Neat's-foot oil 95

65 *Example 6*

- Parts  
Furfuryloxyacetic acid cyclohexylamine salt 2  
Blown neat's-foot oil 98

70 *Example 7*

- Parts  
Tetrahydrofurfuryloxyacetic acid dimethylcyclohexylamine 3  
Water 1  
75 Sperm oil 96

*Example 8*

- Parts  
Tetrahydrofurfuryloxyacetic acid piperidine salt 1-5  
Blown sperm oil 99-95 5

*Example 9*

- Parts  
Furfuryloxyacetic acid morpholine salt 2  
Mineral oil 90 10  
Diethylene glycol ditetrahydrofuroate 8

*Example 10*

- Parts  
Tetrahydrofurfuryloxyacetic acid benzylamine salt 1-5 15  
Blown teaseed oil 99-95

*Example 11*

- Parts  
Teaseed oil 25 20  
Di- $\beta$ -methoxyethyl succinate 70  
Tetrahydrofurfuryloxyacetic acid piperazine salt 5

*Example 12*

- Parts  
Water 80  
Gelatin 5  
Furfuryloxyacetic acid ethylene diamine salt 10  
Tetrahydrofurfuryl tetrahydrofuroate 5 30

*Example 13*

- Parts  
Water 70  
Water soluble cellulose ester 5  
Tetrahydrofurfuryloxyacetic acid triethanolamine salt 20  
Sulfonated olive oil 5

*Example 14*

- Parts  
Tetrahydrofurfuryloxyacetic acid tetramethylammonium hydroxide salt 1-10  
Blown neat's-foot oil 99-90

Any of the above compositions may be applied to the yarn intended for use in circular knitting by means of a bath, wick, spray, roller, pad or any suitable means. The amount of conditioning liquid applied may vary between 5-25% by weight of the yarn. Usually, however, the amount of conditioning liquid applied is about 10-15% by weight of the yarn. Yarn composed of cellulose acetate conditioned as described above gives excellent results when used in the circular knitting process.

As will be apparent from the above examples and description the conditioning agents of our invention may be applied by a wide variety of methods. For example, we may employ the agent as an ingredient of the spinning dope from which the filaments are formed, the amount of the agent so employed depending upon a number of factors, such as the particular cellulose derivative used in making the yarn, the solvent or solvent combination used in making up the spinning solution, and the properties desired in the finished yarn, etc.

If the conditioning agent is to be applied to the yarn after spinning, this may be done by bringing the yarn in contact with a wick, roll, or felt wet therewith, or the liquid may be applied by immersion, spray, or otherwise. The particular point at which the liquid is applied may vary. It may, for example, be applied to the yarn inside or outside the spinning cabinet, between the guide and godet roll, between the godet

5 or other roll or guide and the point of winding and/or twisting. In some cases, the liquid may even be applied to the yarn after winding onto cones, spools, bobbins, or the like or by the so-called "bobbin to bobbin" method. In the case of staple fiber manufacture, the liquid may be applied to the yarn prior to, or after cutting into staple lengths.

10 The amount of the agent so employed will vary widely depending upon the results desired, the specific nature of the material to which the agent is applied, the use to which the yarn is eventually to be put and other factors. For example, in a given case where a cellulose organic acid ester  
15 yarn such as a yarn composed of cellulose acetate, is intended for knitting, about 4 to 25% or more by weight, based on the weight of the dry yarn, may be satisfactory, while if the yarn is intended for weaving, the amount may vary  
20 between about 1 and 5%.

Although in the above examples we have referred primarily to yarn treating compositions containing only the conditioning agent and an oil, other ingredients such as solvents, non-solvents, emulsifying agents, blending agents and the like, may be added within the scope of our invention. Likewise, various dyes or other coloring matter may be included in case it is desired to permanently or fugitively tint or dye the material undergoing treatment.

Although we have found it convenient to illustrate our invention by reference to compositions containing specific percentages of the various ingredients, these percentages may vary widely depending upon the particular purpose for which the composition is intended. For example, if it is desired to control the deelectrifying action of the conditioning agent, the amount of the agent may be adjusted as, for example, by reducing the amount of the agent and correspondingly increasing the amount of oil or other ingredient.

While we have described our invention with particular reference to the treatment of yarns composed of organic derivatives of cellulose such as cellulose acetate, the conditioning agents and formulas described herein are applicable to the conditioning of many other types of cellulose derivative yarns such as those composed of or containing cellulose propionate, cellulose butyrate, cellulose acetate propionate, cellulose acetate butyrate, ethyl cellulose, methyl cellulose, benzyl cellulose and others, as well as to the conditioning of silk, wool, cotton, viscose and other natural or artificial materials.

The term "yarn" as used herein and in the claims is to be understood as including a single filament, a plurality of filaments associated into the form of a thread, either of high or low twist, single or multiple threads associated or twisted together, composite threads composed of a mixture of natural and artificial filaments or a composite thread formed by twisting together individual strands of natural or artificial materials, as well as cut staple fibers produced from natural and/or artificial filaments or threads and spun yarn produced from such staple fibers.

As indicated above, the yarn conditioning agents of our invention are exceptionally good solvents for a wide variety of mineral, blown and unblown, drying and semi-drying animal and vegetable oils such as cottonseed, olive, castor, neat's-foot, sperm and other oils. This enables them to be used with any of such oils in making up a variety of yarn treating formulas of varying composition.

The yarn conditioning agents of our invention also have exceptional value as surface active compounds and as such may be employed as wetting agents, emulsifying and dispersing agents, textile assistants, dye dispersing agents and the like.

The yarn conditioning method and compositions of our invention possess many outstanding advantages. The fundamental and outstanding characteristic of the agents employed in accordance with the invention is their ability to de-electrify yarns, especially those composed of or containing organic derivatives of cellulose such as cellulose acetate and render them amenable to various textile operations, especially operations such as those involved in the manufacture of cut staple fibers, as well as in weaving and knitting. Another outstanding characteristic of these compounds is their exceptional solvent power for a wide variety of mineral, animal, and vegetable oils and their ability to act as lubricating assistants in conjunction with these oils when applied to such yarns. In addition, due to their solubility in water, they may be readily removed from yarns and fabrics by means of the usual aqueous scour baths. By employing the yarn conditioning agents and method of our invention as herein described, one is enabled to obtain highly satisfactory results in the manufacture of yarns and woven fabrics and especially the production from these yarns of cut staple fibers and spun yarn.

What we claim and desire to secure by Letters Patent of the United States is:

1. The method of eliminating the tendency of 35  
yarns, filaments or fibers to accumulate charges  
of static electricity, which comprises applying  
thereto a composition containing as its essential  
anti-static component a salt selected from the  
group consisting of the amine salts of fur- 40  
furyloxy and tetrahydrofuryloxy aliphatic  
acids, said salts having the structural formula



where A is a substituent selected from the group consisting of alkyl groups and hydrogen;  $n$  and  $x$  are small whole numbers at least 1; and B is a substituent selected from the group consisting of the primary, secondary, tertiary and quaternary organic bases and ammonia.

2. The method of eliminating the tendency of yarns composed of or containing organic derivatives of cellulose, filaments or fibers to accumulate charges of static electricity, which comprises applying thereto a composition containing as its essential antistatic component a salt selected from the group consisting of the amine salts of furfuryloxy and tetrahydrofurfuryloxy aliphatic acids, said salts having the structural formula



where A is a substituent selected from the group consisting of alkyl groups and hydrogen;  $n$  and  $x$  are small whole numbers at least 1; and B is a substituent selected from the group consisting of the primary, secondary, tertiary and quaternary organic bases and ammonia. 70

3. The method of eliminating the tendency of yarns composed of or containing cellulose acetate, filaments, or fibers, to accumulate charges of static electricity, which comprises applying

thereto a composition containing as its essential anti-static component a salt selected from the group consisting of the amine salts of furfuryloxy and tetrahydrofurfuryloxy aliphatic acids, said salts having the structural formula



- 10 where A is a substituent selected from the group consisting of alkyl groups and hydrogen;  $n$  and  $x$  are small whole numbers at least 1; and B is a substituent selected from the group consisting of the primary, secondary, tertiary and quaternary organic bases and ammonia.

4. The method of eliminating the tendency of  
yarns composed of or containing cellulose ace-  
tate, filaments, or fibers, to accumulate charges  
of static electricity, which comprises applying  
thereto a composition containing as its essential  
anti-static component a salt selected from the  
group consisting of the amine salts of furfuryl-  
oxy and tetrahydrofurfuryloxy aliphatic acids,  
said salts having the structural formula



- 30 where A is a substituent selected from the group consisting of alkyl groups and hydrogen;  $n$  and  $x$  are small whole numbers at least 1; and B is a substituent selected from the group consisting of the primary, secondary, tertiary and quaternary 35 organic bases and ammonia, and a textile lubricant.

5. The method of eliminating the tendency of yarns composed of or containing organic derivatives of cellulose, filaments or fibers to accumulate charges of static electricity, which comprises applying thereto a composition containing as its essential anti-static component tetrahydrofurfuryl-oxy-acetic acid sodium salt.:

45 6. The method of eliminating the tendency of  
yarns composed of or containing organic derivatives  
of cellulose, filaments or fibers to accumulate  
charges of static electricity, which comprises  
applying thereto a composition containing as  
its essential anti-static component tetrahydro-  
50 furfuryloxyacetic acid triethanol amine salt.

50 7. The method of eliminating the tendency of  
yarns composed of or containing organic derivatives  
of cellulose, filaments or fibers to accumulate  
charges of static electricity, which comprises  
55 applying thereto a composition containing as its  
essential anti-static component tetrahydrofurfuryloxyacetic acid dimethyl cyclohexylamine  
salt.

8. Textile yarns having a lessened tendency to accumulate charges of static electricity, said yarns containing a salt selected from the group consisting of the amine salts of furfuryloxy and tetrahydrofurfuryloxy aliphatic acids, said salts having the structural formula



- 70 where A is a substituent selected from the group consisting of alkyl groups and hydrogen;  $n$  and  $x$  are small whole numbers at least 1; and B is a substituent selected from the group consisting

of the primary, secondary, tertiary and quaternary organic bases and ammonia.

9. Textile yarns composed of or containing organic derivatives of cellulose having a lessened tendency to accumulate charges of static electricity, said yarns containing a salt selected from the group consisting of the amine salts of furfuryloxy and tetrahydrofurfuryloxy aliphatic acids, said salts having the structural formula



where A is a substituent selected from the group consisting of alkyl groups and hydrogen;  $n$  and  $x$  are small whole numbers at least 1; and B is a substituent selected from the group consisting of the primary, secondary, tertiary and quaternary organic bases and ammonia. 15

10. Textile yarns composed of or containing cellulose acetate having a lessened tendency to accumulate charges of static electricity, said yarns containing a salt selected from the group consisting of the amine salts of furfuryloxy and tetrahydrofurfuryloxy aliphatic acids, said salts having the structural formula 20  
25



where A is a substituent selected from the group consisting of alkyl groups and hydrogen;  $n$  and  $x$  are small whole numbers at least 1; and B is a substituent selected from the group consisting of the primary, secondary, tertiary and quaternary organic bases and ammonia. 35

11. Textile yarns composed of or containing cellulose acetate having a lessened tendency to accumulate charges of static electricity, said yarns containing a salt selected from the group consisting of the amine salts of furfuryloxy and tetrahydrofurfuryloxy aliphatic acids, said salts having the structural formula 40



where A is a substituent selected from the group consisting of alkyl groups and hydrogen;  $n$  and  $x$  are small whole numbers at least 1; and B is a substituent selected from the group consisting of the primary, secondary, tertiary and quaternary organic bases and ammonia, and a textile lubricant.

12. Textile yarns composed of or containing organic derivatives of cellulose having a lessened tendency to accumulate charges of static electricity, said yarns containing tetrahydrofurfuryloxyacetic acid sodium salt. 55

13. Textile yarns composed of or containing organic derivatives of cellulose having a lessened tendency to accumulate charges of static electricity, said yarns containing tetrahydrofuryloxyacetic acid triethanolamine salt. 60

14. Textile yarns composed of or containing organic derivatives of cellulose having a lessened tendency to accumulate charges of static electricity, said yarns containing tetrahydrofurfuryl oxyacetic acid dimethyl cyclohexylamine salt. 65

70

JOSEPH B. DICKEY.  
JAMES G. McNALLY.